

## UNITED STATES PATENT OFFICE

2,640,841

REFINING AND BLEACHING OF SUGAR  
CANE WAX

Harold Herbert Hatt, Kew, Victoria, Peter Hermann Alois Strasser, Balwyn, Victoria, and William John Troyahn, Gardiner, Victoria, Australia, assignors to Commonwealth Scientific and Industrial Research Organization, East Melbourne, Victoria, Australia, a body corporate

No Drawing. Application April 17, 1951, Serial No. 221,524. In Australia February 7, 1950

6 Claims. (Cl. 260—423)

1

Our invention relates primarily to the refining of sugar cane wax but refers also to an improved method of bleaching such wax.

It is known that a crude sugar cane wax may be extracted from the clarification or filter cake of sugar cane mills by means of an organic solvent and that a variety of such solvents may be used for this purpose. Depending on the type of cane and the processes used at the sugar mill for processing the cane juices, as well as on the solvents used for extraction, the crude wax contains varying amounts of non-wax components and varying amounts of ash-yielding material, and may be from green-brown to dark brown in colour. Some of the non-wax constituents of the crude wax are soft and fat-like in consistency and confer on the wax a sticky nature. Prolonged presence in the filter-cake also gives rise to a musty odour in the crude wax.

It has been the aim of many investigators to produce from this crude wax a pale, odourless, hard wax, free of the soft fat-like materials and of the ashable matter. It is known that the ashable material can be removed by washing with aqueous mineral acids. Many processes have been described which seek to remove the softer components and the colour of the crude wax by preferential extraction either of the wax or non-wax components in a suitable organic solvent. Other processes seek to remove colour by its adsorption from an organic solvent on to a suitable adsorbent earth.

The main object of our invention is to provide an improved method of removing the undesirable softer and fat-like components and a further object is to provide an improved method of bleaching the refined wax.

According to our invention the crude wax, after it has been freed of mineral matter, if present, by digestion with a mineral acid, is distilled under a pressure of not greater than about 6 millimetres of mercury in an inert atmosphere such as steam, carbon dioxide or nitrogen at a temperature which rises above 250° C. and does not exceed 325° C. and which is maintained within that range until the desired proportion of distillate has passed off. The preferred atmosphere is steam. After treatment in this manner, a hardened dark wax remains as the residue, the undesirable components having passed over

2

with the distillate. This wax is free of objectionable odour. The hard dark wax may then be bleached by chromic acid in sulphuric acid solution to a hard pale wax.

5 In our invention the object is to remove the softer free fatty acids and fat-like components of crude sugar cane wax as distillate. These may comprise 40% of the crude wax. A hard dark wax of low acid value then remains. For 10 this purpose the distillation temperatures used range from 250 to 325° C. and distillation pressure is low, lying preferably between 0.5 and 2.0 mm. of mercury. The hard wax remaining undistilled after this treatment does not suffer serious alteration and possesses approximately the properties of the hard dark wax obtained by the processes of solvent refining examples of which are given by R. T. Balch in "Wax and Fatty Byproducts of Sugar Cane" Technological Report No. 3, Sugar Research Foundation Inc., New York, 1947.

20 The nature of the hard wax can be varied by adjusting the proportion of material distilled. This may be done either by interrupting the distillation or by selecting within the range 250° C.—325° C. at temperature at which only the desired percentage of distillate can distill. Below 25° C. it is not possible to remove the undesirable components except by the use of inconveniently 25 low pressures of the order of 0.01 mm. while above 325° C. the wax is damaged by thermal decomposition. Thus, from an ash-free crude wax initially having an acid value of 45, a melting point of 69–70° C., and a Brinell hardness of 0.50, after removing 8% at 250° C. under a pressure of 1 mm. of mercury, an odourless, dark wax remained having an acid value of 8, a melting point of 73° C. and a Brinell hardness of only 0.77. After 38% of the same wax had been 30 removed at 300° C. under 1 mm. pressure, the residual wax had an acid value of 3, melted at 74° C. and had the much higher Brinell hardness of 2.23.

40 Such a refined wax may be bleached by chromic acid in sulphuric acid solution to valuable hard waxes, which, depending on the amount of chromic acid used, may be pale brown to white in colour and have acid values up to 180.

45 The undesirable softer components of the wax removed by distillation are obtained by this

means in a condition which makes them an attractive by-product. They are pale brown in colour, free of odour, and may be easily collected fractionally by changing the receiver during distillation. Thus, when three fractions were made during a distillation at 1 mm. pressure, they possessed the properties tabulated:

|        | Temperature During Distillation (°C.) | Percent Distilled | Melting Point (°C.) | Acid Value | Saponification Value | Iodine Value | Percent Unsaponifiable |
|--------|---------------------------------------|-------------------|---------------------|------------|----------------------|--------------|------------------------|
| 1----- | Rising to 260....                     | 11                | 40                  | 183        | 190                  | 71           | 9                      |
| 2----- | 260-300-----                          | 11                | 59                  | 77         | 83                   | 70           | 50                     |
| 3----- | 300-----                              | 13                | 60                  | 63         | 75                   | 73           | 70                     |

This shows that the acidic materials are concentrated in the first portions of the distillate and that later portions of the distillate consist largely of neutral material.

The invention is illustrated but is not limited by the following examples.

*Example 1*

Crude sugar cane wax, obtained by extracting a filter cake with a petroleum fraction (Shell X2) at its boiling point, was freed of ashable material by digestion with dilute hydrochloric acid and with water, according to known methods. It then melted at 69-70° C., possessed an acid value of 45, and a Brinell hardness of 0.50.

400 g. of the resultant wax were placed in a 1 litre Pyrex flask fitted with a long neck and a wide delivery tube. The flask was connected to suitable receiving vessels, evacuated to 1 mm. pressure and heated first at 200° C., increasing the temperature during 1 hour to 300° C. Steam was admitted into the flask under the wax at a rate of 2 g. per hour. At the end of 3 hours 30% of the wax had distilled and the distillation was terminated and carbon dioxide or nitrogen was admitted to the distillation flask. The residual, vacuum-hardened wax was odourless, dark brown in colour, melted at 72° C., had an acid value of 6, an iodine value of 37 and a Brinell hardness of 1.78.

The distillate when collected as a whole was a pale brown paste with an acid value of 87 and an iodine value of 79 and melted at 57° C. It could be fractionally collected as above stated.

*Example 2*

100 g. of the vacuum-hardened wax of Example 1 were placed in a flanged 3 litre reaction flask fitted with a horse-shoe stirrer and 100 ml. of 30% w/v. aqueous sulphuric acid, but, preferably, 100 ml. of spent liquor from a previous bleach, were added. The flask was fitted with a reflux condenser and a dropping funnel. The mixture was stirred and the vessel heated in an oil-bath to cause refluxing. Chromic acid (90 g.) was then added continuously over a period of four hours as 833 ml. of a solution containing 108 g. chromic acid and 420 g. sulphuric acid per litre. After heating and stirring a further 3 hours, heating was discontinued and stirring continued until the temperature reached 100° C. After standing, 830 ml. of the spent aqueous

liquors were withdrawn. The wax and remaining liquors were again stirred and heated while a further 550 ml. of the bleaching solution were added in 4 hours. Heating was continued for 8 hours and again the spent liquors were withdrawn when the wax had separated. The solid was washed with cold water, then stirred

and refluxed for 1 hour with 750 ml. of 30% sulphuric acid and again the aqueous liquors drawn off after separating. The wax was then washed 3 times with cold water, once by refluxing for 1 hour with 750 ml. of water, allowed to separate, collected, dried in vacuo at 95° C. and flaked.

This wax was yellow in colour, melted at 76° C., had an acid value of 120, an iodine value of zero and a Brinell hardness of 1.67. It was obtained in a yield of 82 g. (82%).

We claim:

1. A method of refining sugar cane wax, comprising the distilling of undesirable components from the crude wax under a pressure not greater than about 6 millimetres of mercury in an inert atmosphere and at a temperature which rises above 250° C. and does not exceed 325° C. and which is maintained within that range until the desired proportion of distillate has passed off.

35 2. A method of refining sugar cane wax as claimed in claim 1, in which the distillation is carried out in an atmosphere of steam.

3. A method of refining sugar cane wax as claimed in claim 1, in which the distillation is carried out at a temperature of about 300° C.

40 4. A method of refining sugar cane wax as claimed in claim 1, and in which the wax which remains as the residue is bleached by chromic acid in sulphuric acid solution.

45 5. A method of refining sugar cane wax as claimed in claim 1, in which the distillation is carried out under a pressure between 0.5 and 2.0 millimetres of mercury.

60 6. A method of refining sugar cane wax as claimed in claim 1, in which the softer components distilled from the wax are fractionally collected.

55 HAROLD HERBERT HATT.  
PETER HERMANN ALOIS STRASSER.  
WILLIAM JOHN TROYAHN.

References Cited in the file of this patent  
UNITED STATES PATENTS

60 Number Name Date  
2,401,338 Dunmire ----- June 4, 1946

FOREIGN PATENTS

65 Number Country Date  
1,332 Great Britain ----- 1915  
9,105 Great Britain ----- 1893